

Patented Apr. 13, 1926.

1,580,138

# UNITED STATES PATENT OFFICE.

HENRY HARRIS, OF LONDON, ENGLAND.

## TREATMENT OF IMPURE MOLTEN METAL AND METALLIC MASSES.

No Drawing.

Application filed December 11, 1924. Serial No. 755,160.

To all whom it may concern:

Be it known that I, HENRY HARRIS, a subject of the King of Great Britain, and resident of London, England, have invented 5 certain new and useful Improvements in Treatment of Impure Molten Metal and Metallic Masses, of which the following is a specification.

My invention relates to the treatment of 10 impure molten metal and molten metallic masses, and more particularly to the treatment of impure molten lead and other metallic masses containing one or more alloying ingredients, such for example, as arsenic 15 and/or tin with or without antimony. The invention is especially useful for the simultaneous treatment of molten lead containing alloying ingredients and of a spent reagent containing a lead alloying ingredient derived 20 from a previous lead treatment.

It is known according to previous inventions of mine, how to treat molten lead with a reagent comprising caustic alkali, preferably mixed with sodium chloride, and utilizing 25 a suitable oxidizer, to separate from the molten lead various alloying ingredients (my copending application Serial No. 698,279, filed March 10, 1924, and application Serial No. 724,899, filed July 8, 1924, both 30 for refining lead). The alloying ingredients, according to the known inventions, may be removed together or fractionally. In my last said application I have described 35 a process whereby the alloying ingredients arsenic, tin and antimony may be very effectively removed together or fractionally by bringing the molten lead containing the alloying ingredients into intimate contact with a molten reagent mixture of caustic 40 soda and sodium chloride to which is gradually added a limited quantity of a suitable oxidizer such for example as sodium nitrate. According to said process, the amounts of the reagent ingredients and of the oxidizer, 45 and the duration of the treatment of the molten metal for each batch of reagent is so proportioned that said alloying ingredients may be substantially fractionally removed so that the arsenic is eliminated substantially 50 free of tin, the tin being eliminated substantially free of the antimony, and then the antimony is eliminated. The lead and reagent mix are preferably brought into intimate contact by circulating the lead in distributed or sprayed form while maintained at a temperature not exceeding about

500° C. through the reagent mixture until one of the alloying ingredients, for example, arsenic, is removed perhaps with a little tin, then circulating the lead through another batch of reagent until tin is removed perhaps with a little antimony, and then circulating the lead through another batch of reagent until the antimony is totally removed; the arsenic, tin and antimony ingredients being found in the spent reagent mixes in the form of their oxysalts—i. e., sodium oxysalt of arsenic, sodium oxysalt of tin and sodium oxysalt of antimony; or if desired, the arsenic, tin and antimony may be removed together by one operation; or the arsenic and tin with a little antimony may be removed first, then the rest of the antimony may be removed by a subsequent batch of reagent.

While said process is quite efficient in separating said impurities or alloying ingredients from the lead, and more efficient or economical than any other known process, yet a considerable amount of commercial oxidizer is used which is an item of expense. Furthermore, the resulting spent reagents containing caustic soda and an alkali oxysalt of an alloying ingredient have to be treated to recover the caustic alkali for subsequent use, and also to recover the alloying ingredient, the oxygen being lost. It is also a fact that there is a wider market for some lead alloys than for others. For example, there is a better market for antimonial lead than for a tin-antimony lead alloy. Furthermore, the conversion of the oxysalt of antimony to metallic antimony involves considerable expense, and the partial or total loss of the alkali with which it has been combined.

The objects of the present invention are to reduce the cost of the treatment of the impure lead or other suitable metallic masses and of the recovery of the alloying ingredients by (a) reducing the amount of commercial oxidizer required in the treatment of the lead or other metallic masses; (b) reducing the quantity of caustic alkali required in the treatment of lead or other metallic masses; (c) reducing the cost of recovery of the caustic alkali from the spent reagent; (d) reducing the cost of recovery of one or more of the alloying ingredients from the spent reagent; and (e) enriching the lead or other metallic masses with an alloying ingredient which forms an alloy for

which there is a good market, and at the same time eliminating from the lead an undesirable alloying ingredient.

Further objects and advantages of the invention will more fully appear from the following description of certain preferred ways of practicing the invention.

The invention consists in the novel process which is hereinafter described, by way of example, according to said preferred ways of practicing the same, and in the novel features or steps of the process. The invention will be more particularly pointed out in the appended claims.

According to one aspect of this invention, advantage is taken of the underlying principle that certain alloying ingredients, such for example as arsenic, tin and antimony, may be, at least to a large extent, preferentially or fractionally oxidized out of molten lead and other molten metallic masses, to enable the utilization of a spent reagent containing an alkali oxysalt of one or more of said alloying ingredients as an oxidizer in the treatment of molten lead and other suitable metallic masses. For example, if molten lead containing tin and antimony is to be treated by the use of caustic soda, inasmuch as the antimony has less affinity for the oxygen of the oxysalt in the reagent mix than has the tin, if we use in the reagent mix, oxysalt of antimony in the presence of free caustic soda, the antimony will be reduced to metallic antimony which will join any antimony in the lead (or if no antimony is present in the lead the antimony of the oxysalt will join the lead), the oxygen of the oxysalt combining with the more readily oxidizable alloying ingredient, tin, to oxidize the tin and thus separate it from the lead in the form of its alkali oxysalt. Therefore, a spent reagent containing an alkali oxysalt of antimony may be used as an oxidizer for the treatment of lead for the separation of the tin, thus reducing the amount of commercial oxidizer to be added in such treatment.

For example, in utilizing sodium antimoniate as an oxidizer for removing tin from lead, the following equation shows the reaction that is believed to take place:



From this equation it will be seen that if 480 parts by weight of antimony contained in its oxysalt in suspension in caustic soda, be brought into intimate contact with molten lead containing 593 parts of tin this latter will be oxidized and join the caustic mixture as sodium stannate, releasing 480 parts of metallic antimony which will become alloyed with the lead from which the tin has been removed by oxidation.

Similarly, in utilizing sodium antimoniate

as an oxidizer for removing arsenic from lead, the following equation will show the reaction which is believed to take place:



In this case 240 parts by weight of antimony contained in the oxysalt in suspension in caustic soda will effectively remove 150 parts by weight of arsenic contained in molten lead, and this arsenic in the form of alkaline arsenate will replace the antimony oxysalt in the alkaline mixture, while 240 parts by weight of metallic antimony will become alloyed with the lead from which the arsenic has been removed. 80

Similarly again, in using an alkali oxysalt of tin contained in a caustic alkali mixture for removing arsenic from lead, the following formula is believed to represent the reactions:



According to this formula, 593 parts by weight of tin contained in its oxysalt in suspension in caustic soda will remove substantially 300 parts by weight of arsenic from molten lead containing arsenic, in which case 593 parts of tin in metallic form will become alloyed with the lead and replace the arsenic in the lead, and at the same time the arsenic in the form of its alkaline oxysalt will replace in the alkaline mixture the alkali oxysalt of tin. In the treatment, by this invention, of impure metallic masses of low melting point, such for example as the treatment of impure lead, the molten metallic mass as pointed out in my above-mentioned copending applications, is preferably maintained at a temperature not exceeding about 500° C. 100

While these are given as examples of the probable reactions taking place where caustic alkali and in particular caustic soda is used, it will be understood by those skilled in the art that these exact amounts will vary under different practical conditions. It will be further understood that in any case if there are two alloying ingredients to be removed from the lead, a different computation for the oxidizer must be made, and that in any case some other oxidizing agent may be used along with the alkali oxysalt of a lead alloying ingredient to get the proper stoichiometric requirements for the reactions. 110

Besides reducing the amount of commercial oxidizer required, it is possible to thus utilize the total alkali of the spent reagent for the further treatment of lead without having first to recover it from the spent reagent. Another advantage is that it is not necessary to otherwise treat the particular spent reagent containing the oxysalt of 120

antimony for the recovery of the antimony, because the antimony as metal rejoins the molten lead to enrich it as a lead-antimony alloy—antimonial lead, for which there is usually a good market.

5 The invention is useful in a case where there may be a spent reagent containing the oxysalts of arsenic, tin and antimony, for the treatment of lead containing arsenic and/or tin, and antimony, for the separation of the arsenic and/or tin.

10 The invention is useful in such a case regardless of whether the antimony is to be finally removed from the lead or left in the lead as antimonial lead. For example, if we use a caustic alkali reagent containing the alkali oxysalts of arsenic, tin and antimony for the treatment of lead containing arsenic, tin and antimony, the antimony of 15 the reagent will go to join the antimony in the lead and cause the arsenic and tin of the lead to separate out in the form of their oxysalts (assuming always, of course, that the stoichiometric requirements are 20 served). The resulting spent reagent will thus have only the oxysalt of arsenic and tin, the antimony having gone to the lead. If now it is desired to remove the antimony from the lead, the lead will be treated in 25 known manner for this purpose.

30 In the same manner a spent reagent containing an alkali oxysalt of tin may be utilized as an oxidizer for separation of arsenic from the lead in the form of its oxysalt; or the oxysalt of antimony may be thus used to separate from lead both arsenic and tin in the form of their oxysalts; or the alkali oxysalts of antimony and tin may be used to separate the arsenic from 35 the lead.

40 The process holds good for the use of the oxysalt of any alloying ingredient of the lead, as an oxidizer, to separate from the lead any other alloying ingredient or ingredients which have a greater affinity for 45 the oxygen of said oxysalt than has the alloying ingredient of said oxysalt.

Such an alkali oxysalt of the alloying ingredient may be used alone as the oxidizer 50 or in conjunction with some other oxidizing agent such for example as sodium nitrate, according to the amount and composition of said oxysalt on hand, and the quantity and nature of the alloying ingredient of the lead 55 to be treated.

As heretofore, I prefer to use a mixture of caustic soda and sodium chloride as the reagent, because, among other advantages, the sodium chloride renders the reagent mix- 60 more effective as a carrier of alkaline oxysalts.

In carrying out the process, any suitable apparatus may be used, but I prefer to use apparatus such as shown and described in 65 my United States Patent No. 1,465,128,

granted August 14, 1923, for apparatus for refining metals, or as shown in my copending application Serial No. 605,597, filed December 8, 1922, for apparatus for refining or separating metals.

According to another aspect of my invention, if it is desired to treat some molten metallic mass other than impure lead, containing alloying ingredients such for example as those above mentioned, to separate one or more of same, as for example to separate arsenic from molten alloy of tin and arsenic, this can be done by bringing the molten alloy into intimate contact with an alkali oxysalt of tin, the arsenic of the alloy being oxidized and the tin of the oxysalt replacing the arsenic in the alloy. As was above pointed out in the case of treating impure lead, the replacement of arsenic in the alloy by tin is due to the fact that tin has less affinity for the oxygen of the oxysalt in the mixture than has the arsenic; and likewise, as above stated with respect to the treatment of impure lead or lead alloy, the process holds good for the use of the oxysalt of any metal which will combine with the molten metallic mass, as an oxidizer to separate from said metallic mass containing other metallic ingredients, such of them as have a greater affinity for the oxygen of said oxysalt oxidizer than has the metal of said oxysalt oxidizer.

I am aware that in the strictest sense arsenic is not considered as a metal but in metallurgy it is often designated as a metal generally speaking, and I use the words "metal" and "metallic ingredients" herein, in the broader and more general sense, and as including metalloidal substances such as arsenic.

While I have described the invention according to certain preferred ways of carrying out the same, it will be understood by those skilled in the art after understanding my invention, that the invention may be carried out in different ways, and that various changes and modifications may be made therein without departing from the spirit or scope of the invention, and I do not wish to be understood as being limited in the practice of the invention other than as set forth in the appended claims.

Having thus described my invention, what I claim as new and desire to secure by Letters Patent, is:

1. Method of treating a molten metallic mass containing two or more metallic ingredients, for the separation from the mass of one or more of the same by the use of a reagent containing an oxidizer, characterized thereby that as an oxidizer there is added oxysalt of one or more metals which will combine with the metallic mass and which whilst in the mixture, has less affinity for its combined oxygen than has the one or

- more of said metallic ingredients to be removed from the metallic mass.
2. Method of treating a molten metallic mass containing two or more metallic ingredients, for the separation, from the mass of one or more of the same by the use of a reagent comprising caustic soda, characterized thereby that there is added as an oxidizer, oxysalt of one or more metals which will combine with the metallic mass and which whilst in the mixture, has less affinity for its combined oxygen than has the one or more of said metallic ingredients to be removed from the metallic mass.
3. Method of treating a molten metallic mass containing two or more metallic ingredients, for the substitution in the mass of one or more desirable metals for one or more of said metallic ingredients, which comprises bringing into intimate contact said molten metallic mass and a reagent comprising free caustic alkali, to which is added as an oxidizer, oxysalt of one or more desirable metals alloyable with the metallic ingredient or ingredients not to be removed from the metallic mass, said metal of the oxidizer whilst in suspension in the mixture having less affinity for its combined oxygen than has the one or more of said metallic ingredients to be removed from the mass.
4. Method of treating a molten metallic mass containing one or more of the metallic ingredients arsenic, tin and antimony, for separation from the metallic mass of one or more of said metallic ingredients, which comprises bringing into intimate contact said molten metallic mass, a reagent comprising caustic soda, and oxysalt of one or more of said metallic ingredients which last metallic ingredient or ingredients whilst in the mixture has less affinity for its combined oxygen than has the one or more other of said metallic ingredients to be removed from the mass.
5. Method of treating a molten metallic mass containing one or more of the metallic ingredients arsenic, tin and antimony for separation from the metallic mass of one or more of said metallic ingredients, which comprises bringing into intimate contact in the presence of free caustic alkali, said molten metallic mass and oxysalt of one or more of said metallic ingredients, which last metallic ingredient or ingredients whilst in suspension in the mixture has less affinity for its combined oxygen than has the one or more other of said metallic ingredients to be removed from the mass.
6. Method of treating molten lead for separation therefrom of one or more ingredients alloyed therewith, which comprises using as an oxidizer for one or more of the alloying ingredients an alkali oxysalt of a different lead alloying ingredient from the one or ones to be removed.
7. Method of treating molten lead for separation therefrom of one or more ingredients alloyed therewith, which comprises bringing into intimate contact the molten lead and a mixture containing free caustic alkali and an oxysalt of another lead alloying ingredient which will effect the elimination from the lead of said first alloying ingredient or ingredients.
8. Method of treating molten lead for separation therefrom of one or more ingredients alloyed therewith, which comprises bringing into intimate contact the molten lead and a reagent containing caustic alkali and an oxysalt of another lead alloying ingredient which will effect the elimination from the lead of said first alloying ingredient or ingredients by oxidation.
9. Method of treating molten lead for separation therefrom of one or more ingredients alloyed therewith, which comprises bringing into intimate contact the molten lead and a reagent comprising caustic soda and an oxysalt of a lead alloying ingredient which whilst in the mixture has less affinity for its combined oxygen than has the alloying ingredient to be removed from the lead.
10. Method of treating molten lead for separation therefrom of one or more ingredients alloyed therewith, which comprises bringing the molten lead into intimate contact with a reagent comprising caustic alkali, sodium chloride and an oxysalt of an alloying ingredient which whilst in the mixture has less affinity for its combined oxygen than has the alloying ingredient to be removed from the lead.
11. Method of treating molten lead for separation therefrom of one or more ingredients alloyed therewith, which comprises bringing into intimate contact the molten lead with a reagent comprising an oxysalt of a lead alloying ingredient in suspension in caustic alkali and which last alloying ingredient whilst in the mixture has less affinity for its combined oxygen than has the alloying ingredient or ingredients to be removed from the lead.
12. Method of treating molten lead for separation therefrom of one or more ingredients alloyed therewith, which comprises bringing the molten lead while maintained at a temperature not exceeding about 500° C. into intimate contact with a molten reagent comprising molten caustic alkali, and gradually adding as an oxidizing agent an alkali oxysalt of a lead alloying ingredient, which last alloying ingredient whilst in the mixture has less affinity for its combined oxygen than has the alloying ingredient or ingredients to be removed from the lead.
13. Method of treating molten lead for

- the separation of an ingredient alloyed therewith, which comprises separating said alloying ingredient in the form of its oxysalt by treating the molten metal with caustic alkali and an oxidizer comprising an oxysalt of a lead alloying ingredient not so readily separable from the molten lead as is the alloying ingredient to be removed.
14. Method of treating molten lead for the separation therefrom of one or more ingredients alloyed therewith, which comprises treating the molten lead with a reagent comprising caustic alkali and a suitable oxidizer whereby a mixture comprising caustic alkali and one or more oxysalts of said alloying ingredients are derived, and using said derived mixture as an oxidizer in the treatment of a further batch of lead for the removal therefrom of a lead alloying ingredient having greater affinity for the oxygen of said oxysalts in the reagent mixture than has the alloying ingredient of said oxysalt.
15. Method of treating molten lead for the separation therefrom of one or more ingredients alloyed therewith, and of simultaneously treating a mixture comprising caustic alkali and an oxysalt of a lead alloying ingredient derived from the refining of lead, to reduce and separate said alloying ingredient from said oxysalt and free the alkali for further use, which comprises bringing into intimate contact said molten lead and
- said mixture containing caustic soda and an alkali oxysalt of an alloying ingredient, which last ingredient while in the mixture has less affinity for its combined oxygen than has the alloying ingredient to be removed from the lead, whereby said oxysalt of the mixture will become decomposed, its alloying ingredient going to the lead in metallic form, its oxygen combining with the more readily oxidizable alloying ingredient of the lead oxidizing said alloying ingredient, and its alkali base combining with the said oxidized alloying ingredient.
16. Method of treating molten lead for the separation therefrom of an undesired alloying ingredient and for the enriching of the lead with another alloying ingredient, which comprises bringing into intimate contact the molten lead containing the undesired alloying ingredient, free caustic alkali and an oxysalt of an enriching alloying ingredient, which ingredient whilst in the mixture has less affinity for its combined oxygen than has the undesired alloying ingredient.
17. Method of separating arsenic from a molten arsenic tin alloy, which comprises bringing said alloy into intimate contact with a reagent containing an alkali oxysalt of tin.

In testimony whereof I have signed my name to this specification.

HENRY HARRIS.